

J. H. PAYNE.

PROCESS OF MAKING ALKALI CHROMATE SOLUTIONS.

APPLICATION FILED AUG. 26, 1911.

1,081,625.

Patented Dec. 16, 1913.



Inventor

J. H. Payne.

Witnesses

Witnesses  
J. M. Fowler Jr.  
Ellen Horodine

၃၃၁

A. P. Greeley

Attorney

# UNITED STATES PATENT OFFICE.

JAMES H. PAYNE, OF YORKTOWN, VIRGINIA, ASSIGNOR TO FRED E. GIGNOUX, OF CAPE ELIZABETH, MAINE.

## PROCESS OF MAKING ALKALI-CHROMATE SOLUTIONS.

1,081,625.

Specification of Letters Patent. Patented Dec. 16, 1913.

Application filed August 26, 1911. Serial No. 646,248.

To all whom it may concern:

Be it known that I, JAMES H. PAYNE, a citizen of the United States, residing at Yorktown, in the county of York and State 5 of Virginia, have invented certain new and useful Improvements in Processes of Making Alkali-Chromate Solutions, of which the following is a specification.

My invention relates to a process of treating 10 chromium ore by subjecting such ore mixed with suitable alkali or alkaline earth salts, hydroxids or oxids to an oxidizing heat to produce chromates soluble in water, and the invention has for its object to produce 15 a process which will be characterized by rapidity of action, completeness of reaction produced, and reduced cost of operation.

In the process of treating chromium ores 20 referred to the sesquioxide of chromium of the ore unites with the alkali or alkaline earth element or elements and with oxygen from the heated gases, to form chromates soluble in water. The operation has heretofore been 25 carried on in stationary reverberatory furnaces involving heavy labor expense and large consumption of fuel. Moreover the yield of soluble chromate from the ore so treated is seldom over 80 per cent. of the 30 theoretical.

The novelty of my invention consists essentially in the use of a particular form of furnace for the treatment of the ore and in the proportioning of the substances forming 35 the raw mixture by which a proper physical condition of the material is secured and maintained during the furnacing operation. Instead of a stationary furnace I employ a rotating cylinder suitably lined, 40 slightly inclined toward the firing end. The raw mixture is fed into the cylinder at the cool end and slowly works its way through to the firing end, being constantly agitated by the rotation of the cylinder, receiving its 45 heat and oxygen from the heated gases and by proper regulation of the speed of rotation of the cylinder and the condition and temperature of the gases forms at the point of incipient fusion into porous rounded or 50 irregular shaped sintered masses ranging in size from that of coarse sand to nodules several inches in diameter. These sintered masses or "clinkers" contain under proper

conditions from 90 to 95 per cent. of the soluble chromates theoretically possible to be produced.

The drawing is a longitudinal elevation partly in section of an apparatus adapted to carry out my invention.

In the drawing which is to be understood 60 as illustrative merely and not as in any way restricting the invention to the use of the particular apparatus shown, A represents a source of gaseous fuel supply here indicated as a gas producer from which a suitable pipe 65 A' A<sup>2</sup> leads through an opening B in a movable firing hood C to the interior of the cylinder D. The opening B is of larger diameter than the exterior diameter of the pipe A<sup>2</sup> so as to permit air to be drawn in 70 to mix with the gas and support combustion. The firing end of the cylinder D is closed by the hood C and its other end opens into a chamber D' from which leads the usual stack or chimney D<sup>2</sup>. Arranged within the chamber D' is a feeding device here shown as a screw conveyer E arranged to discharge into the open end of the cylinder D. The conveyer should, of course, be protected against injury from heat in any convenient way as by a water jacket. The conveyer E is supplied with the raw mixture by a second screw conveyer F which takes it from a bin G. H is a discharge spout for the clinker carried by the hood C.

The cylinder D is supported on an inclination as shown, the firing end being lower than the other end, in the usual way by roller bearings I. I. on which rings I' I' 85 rest and is rotated by means of a pinion K 90 in mesh with a toothed ring K'.

The mixture fed to the rotating cylinder may consist of any of the well known mixtures used in the production of soluble chromates provided the point of incipient fusion 95 is higher than the temperature at which the reaction proceeds speedily. Where sodium is the principal reactive alkaline element, the temperature necessary for a speedy reaction lies between 900° C. and 1200° C. 100 Where potassium is the principal reactive alkaline element this temperature is much lower. The control of the point of incipient fusion is secured by adding lime or other refractory basic material in sufficient quantity 105 to produce the desired effect. An example

of a properly proportioned raw mixture would be 100 parts chrome iron ore (50%  $\text{Cr}_2\text{O}_3$ ) 70 parts soda ash, and 100 parts quick lime.

5 It is essential that sufficient lime or other refractory basic material be added to prevent actual fusion during the furnacing operation because this invariably results in a low yield of soluble chromate. The point of 10 incipient fusion must not be exceeded in order that the masses as they form may remain porous thereby insuring the entrance of the oxidizing gases in the furnacing operation and the leaching solutions in the subsequent leaching operation.

15 The raw mixture may be fed in the form of a slurry in which form a more intimate mixture of the ingredients than can be secured in a dry mixture, is made possible, 20 thereby producing a higher yield and reducing the tendency to ball up. The tendency to ball up is also lessened by the use of limestone in the mixture.

25 It is important that the gases be highly oxidizing and that they move at a high speed. Any kind of fuel may be used either gaseous or liquid or coal and oil, provided precautions are taken to burn them under oxidizing conditions with large excess of air.

30 It will, of course, be understood that the raw mixture is fed continuously into the end of the rotary cylinder and as the cylinder rotates the material will be constantly agitated and by reason of the inclination of the cylinder will move toward the firing end and as it moves toward the firing end will be subjected to an increased degree of heat.

35 It will, of course, be understood that the clinker formed in the furnacing operation above described is subsequently leached to 40 extract the chromate.

Having thus described my invention what I claim is:

1. The process of making an alkali chromate solution which consists in passing a 45 mixture of chrome iron-ore, a basic refractory material and an alkaline material through an inclined rotary cylinder in a direction toward its lower end against a current of oxidizing gases moving toward the higher 50 end of the cylinder and heated to a temperature such as to heat the mixture to a point not exceeding that of incipient fusion, and leaching the resultant porous nodules.

2. The process of making an alkali chromate solution which consists in passing a mixture of chrome iron ore, lime and soda ash through an inclined rotary cylinder in a direction toward its lower end against a current of oxidizing gases moving toward 60 the higher end of the cylinder, and heated to a temperature such as to heat the mixture to a point not exceeding that of incipient fusion, and leaching the resultant porous nodules.

6. 3. The process of making an alkali chromate solution which consists in passing a wet mixture of chrome iron ore, a basic refractory material and an alkaline material through an inclined rotary cylinder in a 70 direction toward its lower end against a current of oxidizing gases moving toward the higher end of the cylinder and heated to a temperature such as to heat the mixture to a point not exceeding that of incipient 75 fusion, and leaching the resultant porous nodules.

JAMES H. PAYNE.

Witnesses:

GEORGE N. WISE,  
W. S. CADWELL.